

# UNITED STATES PATENT OFFICE.

GUILLAUME WEBER, OF HAYANGE, FRANCE, ASSIGNOR TO SOCIETE LES PETITS FILS  
DE FRANCOIS DE WENDEL ET CIE., OF PARIS, FRANCE.

## EXPLOSIVE.

1,375,243.

Specification of Letters Patent. Patented Apr. 19, 1921.

No Drawing.

Application filed September 27, 1919. Serial No. 326,973.

To all whom it may concern:

Be it known that I, GUILLAUME WEBER, citizen of the Republic of France, residing at Hayange, Lorraine, France, have invented new and useful Improvements in Explosives, of which the following is a specification.

It has already been proposed to use explosives depending on the action of liquid air and composed of a combustible metallic powder and a combustible organic substance capable of absorbing liquid air. Aluminium is chiefly adapted for use as a combustible metallic powder but recourse may also be had to magnesium, antimony, silicon and also to iron in the form of a fine powder. It is not always easy to get aluminium, magnesium, antimony and silicon in powdered form or the above materials may be too expensive; on the other hand iron may be easily obtained and at a low cost.

This invention consists also in substituting for the combustible powders indicated above powders or dust coming from the furnaces of metallurgical plants (blast furnace dust), which contain some other combustible materials. Powders coming from blast furnaces possess a certain absorbing power and they might form an explosive with liquid air but it is more advantageous to add an additional combustible absorbent such as sawdust, cotton or coal.

The power of the explosive composed of liquid air, a combustible absorbing substance and blast furnace dust may be augmented

by the addition of combustible metallic powders such as aluminium, magnesium, etc., which are mixed with the other ingredients used or arranged separately.

For the purpose of augmenting the breaking or disruptive effect, hydrocarbons in a solid or liquid state may be added.

The firing of the above explosive inclosed in cartridges may be effected by means of any desired primers.

Having now described my invention what I claim as new and desire to secure by Letters Patent is:

1. An explosive containing a combustible organic substance adapted to absorb liquid air, and blast furnace dust.

2. An explosive containing a combustible organic substance adapted to absorb liquid air, blast furnace dust and combustible metallic powders.

3. An explosive containing a combustible organic substance adapted to absorb liquid air, blast furnace dust, combustible metallic powders and hydrocarbons.

4. An explosive composed of a combustible organic substance adapted to absorb liquid air, blast furnace dust, hydrocarbons and liquid air.

In testimony whereof I have signed my name to this specification in the presence of two subscribing witnesses.

GUILLAUME WEBER.

Witnesses:

JEAN DEMORY,  
EDOUARD FABER.